

# UNITED STATES PATENT OFFICE.

EDMUND A. S. CLARKE, OF CHICAGO, ILLINOIS.

## PROCESS OF PRODUCING SPIEGEL OR SIMILAR METALLIC ALLOY.

SPECIFICATION forming part of Letters Patent No. 604,728, dated May 31, 1898.

Application filed November 28, 1894. Serial No. 530,238. (No specimens.)

*To all whom it may concern:*

Be it known that I, EDMUND A. S. CLARKE, residing at Chicago, in the county of Cook and State of Illinois, have invented certain new and useful Improvements in the Process of Producing Steel by the Bessemer Converter or Open-Hearth Furnace; and I do declare the following to be a full, clear, and exact description of my invention sufficient to enable others skilled in the art to which my invention pertains to practice the same.

In the Bessemer and open-hearth processes of steel manufacture as at present generally practiced the final stage is the addition to the more or less completely decarbonized molten metal within the converter or open-hearth furnace of carbonized manganese-ferous iron, usually spiegeleisen, (or "spiegel," as it is commonly termed,) in definite proportions, so as to communicate to the mixture the desired amount of carbon and of manganese and supplement, if necessary, the percentage of silicon. The usual method of producing the spiegel consists in charging a blast-furnace with the manganese-ferous ore from which it is to be made, and from time to time the furnace is tapped and the metal run out into pigs, as in ordinary blast-furnace operation. It is found that from one cause or another (such as a leaky twyer or the like) the percentage of manganese and silicon contained in the pigs will frequently vary to a considerable extent not only in the pigs produced at different heats or casts from the same furnace, but even a very material variation in the manganese and silicon content is often found in pigs obtained from different parts of the same cast or heat. The pigs thus produced are remelted in a cupola; but owing more especially to the variations in the manganese and silicon contents above noted it is the practice to analyze the pigs and sort and stack them in separate piles, so that the cupola may be charged with such pigs as contain the proper amount of manganese and silicon necessary to give the desired percentages in the spiegel that is to be delivered to the converter or open-hearth furnace in order to impart the predetermined amount of carbon and manganese and silicon to the charge. A number of serious objections exist to this common method of producing steel in the Bessemer

converter or open-hearth furnace, considered as an entirety. In the first place the time and labor required in casting the melted spiegel into pigs, in transporting and handling these pigs, the fuel, labor, and repairs incident to melting the pigs in a cupola, and particularly the loss of manganese and silicon by oxidation in the remelting of the pigs within the cupola constitute a serious objection. Again, it is often desired on very short notice to change the grade or character of the steel to be produced, which is effected by a corresponding change in the grade or character of the spiegel to be used, (the grade being determined by the manganese and silicon contents,) and inasmuch as it is often impracticable to effect this change of the grade or character of the spiegel produced by the cupola with any degree of certainty within the desired time a serious inconvenience in the operation of the plant frequently results. Yet notwithstanding these objections this method above mentioned is still followed.

Indeed, although it may be practically possible to use spiegel direct from the smelting-furnace as a recarburizing addition to the charge of a Bessemer converter or open-hearth furnace in plants at which sudden changes in the grade or character of the spiegel are not required, still at many plants the differences in the percentages of manganese, carbon, silicon, or the like called for by the specifications for different work to be done render it important that corresponding changes in the grade or character of the spiegel shall be made on very short notice, since otherwise serious delay in operation may result.

In modern practice of steel-making the present specifications for carbon, silicon, and manganese in the steel are so rigid and exact and the limit of variation allowed so slight that if the spiegel vary considerably either in manganese or silicon, or both, it cannot be used, variations from the predetermined percentage of manganese being specially objectionable. Yet a desired change in the grade or character of spiegel from a blast-furnace cannot be made with certainty in less than from twelve to twenty-four hours.

Recognizing the desirability of so improving the process of producing steel in the Bessemer converter or open-hearth furnace that

the necessity of casting the spiegel into pigs and subsequently remelting such pigs in a cupola may be avoided, while at the same time enabling the desired changes in the grade 5 and character of the finished product of the converter or open hearth to be quickly and economically effected, I have devised the improvements in the Bessemer or open-hearth processes of producing steel hereinafter described, and particularly defined in the claims 10 at the end of this specification.

In the preferred manner of practicing my invention a blast-furnace of usual or suitable construction is burdened so as to produce a 15 spiegel of such manganese content that even in the greatest ordinary variation of product from the normal product of the furnace the manganese will still remain higher than the highest manganese percentage that it is proposed to use in the spiegel to be delivered to the Bessemer converter. The smelted spiegel tapped from the furnace will be delivered into a ladle or other vessel, and thereby transported to a mixing-chamber of suitable construction—such, for example, as is employed 20 at various steel-works in this country for receiving and mixing the charges of pig metal from the blast-furnaces preparatory to the delivery of such metal to the converters. The 25 spiegel thus tapped from the furnace and with the percentages of its constituents properly determined will have added thereto in the mixing-chamber such quantities of pig-iron or other iron silicon alloy either direct from a blast-furnace or from a cupola (or both) as 30 will give the desired percentages of manganese, carbon, and silicon in the final mixture. If the mixture thus obtained by adding pig-iron to the metal from the spiegel-furnace is 35 found to contain the desired percentage of manganese, silicon, and carbon, it will be tapped from time to time from the mixing-chamber and delivered to the converters or open hearths at the end of the "blow" in 40 usual manner. If it be found, however, that the molten mass of metal within the mixing-chamber is still too high in manganese, more pig-iron of the proper silicon content will be added, whereas if it be found that the metal within the 45 mixing-chamber is too low in manganese then additions of spiegel direct from the spiegel-furnace or from a cupola and containing a higher percentage of manganese will be made in order to raise the manganese percentage of 50 the metal in the mixing-chamber to the desired point. Should the spiegel delivered from the spiegel-furnace be found to be too high or too low in the silicon content to give the desired amount of silicon in the mass of 55 metal within the mixing-chamber, then further additions of spiegel containing excess of manganese will be delivered to the mass within the chamber until the manganese percentage of the metal within the chamber is 60 raised above the desired point, after which pig-iron having a proper silicon content will be added, so as to dilute the mixture until the 65

proper percentages of manganese and silicon are obtained. A spiegel having the desired content of silicon, manganese, and carbon 70 having been thus obtained, a proper quantity thereof will be introduced into the converter or open hearth at the end of the blow or refining operation in the usual manner. Hence it will be seen that by my process not only is 75 the necessity of casting the spiegel into pigs and subsequently remelting such pigs in a cupola avoided, but by my invention the desired changes in the grade or the character of the product of the converter or open hearth 80 can be readily and economically effected by varying the grade or character of the spiegel while it is still in the molten condition in which it comes from the blast-furnace.

Let it be assumed, for illustration, that the 85 desired grade of spiegel is to contain sixteen per cent. manganese and 1.70 per cent. silicon and there is delivered to the mixing-chamber from the blast-furnace, say, forty thousand pounds of spiegel containing twenty-four per cent. manganese and 1.50 per cent. silicon. To get the desired mixture, I would add twenty thousand pounds of pig-iron containing 2.10 per cent. silicon. From this total amount of sixty thousand pounds there may be used 90 by the time the blast-furnace casts spiegel again, say, forty thousand pounds, leaving twenty thousand pounds. I get from the furnace by this cast, say, forty thousand pounds of spiegel containing twenty-five per cent. 95 manganese and 1.60 per cent. silicon. This gives a mixture in the mixing-chamber of sixty thousand pounds containing twenty-two per cent. manganese and 1.63 per cent. silicon. To bring this to the desired composition, I add 100 twenty-two thousand five hundred pounds of pig-iron containing 1.88 per cent. silicon, making in all eighty-two thousand five hundred pounds of the mixture. From this I use, say, forty-two thousand five hundred pounds, 105 and then desire to change to a mixture containing twelve per cent. manganese and 1.80 per cent. silicon. To do this, I add thirteen thousand three hundred and thirty-three pounds of iron containing 2.10 percent silicon, 110 making fifty-three thousand three hundred and thirty-three pounds of the desired mixture. I use, say, from this mixture until there are twenty thousand pounds remaining and then desire to change back to the first mixture 115 of sixteen per cent. manganese and 1.70 per cent. silicon; but at such time it may be found that the furnace is making spiegel containing twenty-two per cent. manganese and 1.40 per cent. silicon. Of this, to obtain the 120 desired manganese in the mixture, I would need thirteen thousand three hundred and thirty-three pounds, but this would give but 1.66 per cent. silicon and only thirty-three thousand three hundred and thirty-three pounds 125 of mixture. I would therefore take the entire cast, say forty-five thousand pounds, which would give sixty-five thousand pounds 130 of a mixture containing 18.92 per cent. man-

ganese and 1.38 per cent. silicon. To bring the mixture to required manganese and silicon, I would then add eleven thousand eight hundred and seventy-five pounds of iron containing 2.67 per cent. of silicon, making a total of seventy-six thousand eight hundred and seventy-five pounds of mixture. It is evident that there may from time to time arise occasions when the spiegel or iron available from the blast-furnace may not be suitable for these additions. In such an event spiegel or iron of the proper grade would have to be melted in a cupola; but these occasions would be rare in normal working of the blast-furnaces, and the advantages and economies resulting from this process would be but slightly affected thereby.

It is manifest that by my improved process above described not only is a great saving effected by avoiding the remelting of the spiegel in a cupola, but I am enabled to change the character or grade of the spiegel upon very short notice, and even between heats of the converter or open hearth, so that a very material saving in the practice of producing steel by the Bessemer or open-hearth processes is effected.

While my invention has been defined more especially with a view to the use of spiegel, it is manifest that it may be followed in the use of other alloys suitable for additions to the charge of a Bessemer converter or open-hearth furnace. So, also, it is obvious that modifications in the precise practice of my invention as hereinbefore defined may be made without departing from the spirit of the invention. Thus, for example, if it is desired to suddenly change the character of the spiegel that is to be delivered to the charge of a Bessemer converter or open-hearth furnace and to use but a very small quantity of such changed mixture—as, for example, in running a few heats only of the converter or open-hearth furnace—then it would not be necessary to change the character of the entire mass of metal within the mixing-chamber, particularly if the chamber be of large capacity. In such case I would tap from my mixing-chamber into a suitable ladle a quantity of the spiegel and would then add to the ladle a suitable quantity of molten pig-iron or spiegel, or both, sufficient to give to the mass of molten mixture within the ladle the precise character or grade of spiegel desired for the few heats of the converter or open-hearth furnace that are to be made with such spiegel. Under such conditions the ladle would then serve as a mixing-chamber; but manifestly the broad feature of my invention would be followed, because in such ladle, thus serving as a mixing-chamber, the character of the spiegel would be varied by the additions of molten metal necessary to give the desired grade or character to the spiegel that was to be added to the converter or open-hearth furnace.

I have alluded in this specification to the

possibility of employing spiegel direct from the spiegel-smelting furnace as a recarburizing condition to the charge of a Bessemer converter or open-hearth furnace; but I do not wish this to be understood as of my invention. In its broad feature my invention consists in improving the Bessemer or open-hearth process of producing steel by modifying or changing the grade or character of the spiegel from the smelting-furnace and while still in the molten condition in which it is delivered from such furnace—*i. e.*, without remelting—in order to better adapt it for use and in order to enable changes in the grade or character of the spiegel required by different kinds of work to be quickly effected and thereafter, while still in such molten condition, adding such spiegel after the blow or refining operation to the charge of the converter or open hearth. While I have described what I regard as the preferred manner of carrying out this broad feature of invention, I do not wish the invention to be restricted to such precise process, since manifestly variations in details of process treatment may be made without departing from the spirit of the invention.

Having thus described the invention, what I claim as new, and desire to secure by Letters Patent, is—

1. The hereinbefore - described improvement in the process of producing steel in a Bessemer converter or open-hearth furnace, that consists in charging the converter or open hearth with molten iron and thereafter delivering to said converter or open hearth, after the refining operation, a proper quantity of a molten metallic alloy (such as spiegel) while still in the molten condition in which it is received from the smelting-furnace (*i. e.*, without remelting) suitable additions in proper quantity being made to said molten metallic alloy, before its delivery to the converter, in order to impart to said alloy a character that shall adapt it for use as an addition, after said refining operation to the charge of the converter or open-hearth furnace.

2. The hereinbefore - described improvement in the process of producing steel in a Bessemer converter or open-hearth furnace, that consists in smelting a manganeseiferous ore adapted to produce a metallic alloy for an addition to the charge of said converter or open-hearth furnace, then delivering said alloy in molten condition from the smelting-furnace into a suitable mixing-chamber and therein adding to the charge of the mixing-chamber a further quantity of molten metal containing one or more agents (such as manganese, silicon, carbon, or the like) in proper quantity to give to the mass of metal within the mixing-chamber the desired grade or character, and thereafter adding a quantity of said molten metallic alloy from said mixing-chamber to the mass of metal within the Bessemer converter or open-hearth furnace at the end of the refining operation.

3. The hereinbefore - described improvement in the process of producing steel in the Bessemer converter or open-hearth furnace, that consists in charging a smelting-furnace with ore sufficiently high in manganese to give to the smelted metal a percentage of manganese in excess of that required to be delivered to the converter or open hearth as a rebarburizing addition at the end of the refining operation, then tapping the smelted metal from the furnace and delivering it into a suitable mixing-chamber and therein adding to it molten iron of proper silicon content

and in proper quantity to bring the manganese and silicon contents of the mass of metal within the mixing-chamber to the desired percentages, and finally adding a quantity of said molten metal from said mixing-chamber to the mass of metal within the Bessemer converter or open-hearth furnace at the end of the refining operation.

EDMUND A. S. CLARKE.

Witnesses:

GEORGE P. FISHER, Jr.,  
ALBERTA ADAMICK.